

March 20, 1945.

2,371,604

J. B. BRENNAN  
METHOD OF AND APPARATUS FOR MAKING METAL  
WIRE, ROD, STRIP AND THE LIKE  
Filed Aug. 16, 1941



INVENTOR  
JOSEPH B. BRENNAN  
BY *Borworth & Sessions*  
ATTORNEYS

## UNITED STATES PATENT OFFICE

2,371,604

METHOD OF AND APPARATUS FOR MAKING  
METAL WIRE, ROD, STRIP, AND THE LIKE

Joseph B. Brennan, Euclid, Ohio

Application August 16, 1941, Serial No. 407,199

8 Claims. (Cl. 22—57.2)

This invention relates to the making of metallic wire, rod, strip, and the like, and particularly to the formation of metals into such shapes directly from the molten metal. Insofar as common subject matter is concerned, this application is a continuation in part of my copending application Serial No. 293,341, filed September 5, 1939.

Wire, rod, strip, and the like, are ordinarily produced by expensive and relatively slow rolling or drawing processes or, in the case of rods and some of the soft metals, by extrusion at extremely high pressures through dies. Both types of processes require very expensive equipment and the many operations required add greatly to the cost of the finished product. It is the general object of my invention to provide a method and apparatus for making such shapes wherein the shapes are formed directly from the molten metal, thus eliminating the many rolling and drawing steps or the expensive extruding operation heretofore required.

Briefly, a preferred form of my invention contemplates the melting of metal ingots (the invention is described herein with particular reference to aluminum, but it is to be understood that my invention is not limited to any particular metal or alloy) in an apparatus such as described in my copending application aforesaid and comprising a crucible heated by electricity or other means within a pressure chamber. Thus considerable pressure may be exerted on the molten metal without applying destructive forces to the crucible because of the fact that the pressures are equalized on both the outside and the inside of the crucible. From the crucible the metal is led beyond the interior of the pressure chamber in molten condition preferably through a passageway, the temperature of which can be controlled with a reasonable degree of accuracy. The passageway terminates in a cooling zone wherein the metal is solidified, the passage through the cooling zone being of a shape to form the molten metal into the desired configuration. This cooling zone, as distinguished from an ordinary extrusion die, is of considerable length with the result that the metal enters into the cooling zone while molten, and while still in the molten state is caused to assume the desired cross-sectional shape. As the metal moves along it is gradually cooled, becoming plastic and then solid before its discharge. As most metals contract upon solidification and cooling, there is not excessive friction between the solid metal and the walls of the cooling passageway so that the metal may be moved through the passageway

without requiring excessive pressure or resulting in excessive wear on the cooling passageway. The discharge of the metal may be assisted by a pair of rolls. Preferably the point of discharge is shielded by a reducing flame, and the metal may be cooled by water or steam shortly after it is discharged. Preferably substantial pressures are employed in order to improve the character of the metal produced by my method, but these pressures are far below those required for the usual extrusion processes. To avoid interruption of the operation of the apparatus, a pressure trap is provided for charging the crucible with molten metal.

- 15 My method in one sense may be considered as a continuous pressure casting and drawing method wherein the molten metal may be continuously fed into a mold, permitted to solidify in the mold, and the solidified metal continuously withdrawn therefrom. The method is especially adapted for the production of wire, the production of rods having shapes similar to those of rods produced by present day extrusion methods, the production of tubing, and the production of strip. My method contemplates that in the manufacture of material designed for some services, it will be desirable to subject the wire, rod, tubing or strip produced by my method to further mechanical reduction as by rolling or drawing, particularly in instances where it is important to have high strength in the ultimate product or where very fine wires or thin strips are desired. However, for many purposes my method will produce metal suitable for use without further treatment. For example, in the production of electrolytic condensers, processes of spraying aluminum are widely used. The spraying step as ordinarily practiced requires the use of a spray gun in which aluminum wire is melted. This wire should be of high purity and of substantially uniform diameter, but otherwise its physical characteristics are not important. For such purposes, my method and apparatus provides a convenient and economical means of producing 30 aluminum wire which is particularly advantageous today in view of the fact that the production of aluminum wire by conventional methods is not sufficient to meet the needs of industry and of national defense.
- 35 Referring to the drawing in which a preferred form of apparatus for carrying out my invention is shown somewhat diagrammatically, Fig. 1 illustrates a transverse section through the entire apparatus; Fig. 2 is a section through the cooling zone as indicated by the line 2—2 of Fig. 1; Fig. 3
- 40
- 45

is a section illustrating the rolls preferably employed to assist in withdrawing the solid material from the cooling zone as indicated by the line 3-3 of Fig. 1; and Fig. 4 is a detail, on an enlarged scale, showing the pressure seal for the wires that carry the heating current.

As shown somewhat diagrammatically in the drawing, a preferred form of apparatus may include a pressure chamber and crucible constructed generally in accordance with my copending application aforesaid and preferably comprising a cylindrical pressure chamber 10 having a bottom portion 11 and a top closure member 12 securely bolted thereto as by bolts 14 and 15 respectively, gaskets 16 and 17 being employed to provide tight joints. To prevent the pressure chamber from becoming overheated, it is preferably water-jacketed as indicated at 18, 19 and 20, or other suitable cooling means may be employed. Water or other cooling liquid may be supplied to the water jacket members through an inlet pipe 21 and discharged through the pipe 22. By this means excessive heating of the pressure chamber and consequent weakening thereof may be eliminated. This construction is particularly advantageous in conjunction with metals or alloys of higher melting points such as ferrous materials, for example, but is not as necessary in conjunction with aluminum or other metals or alloys of relatively low melting points.

The molten metal to be discharged under pressure is contained in a crucible indicated generally at 25 and supported within the pressure chamber in any convenient manner as by rails 26 resting on upstanding bosses 27 extending from the bottom member 11 of the chamber. The crucible preferably includes a metallic shell portion 28 having a depending portion 29 extending to the bottom of the container. The crucible is provided with a lining 30 of refractory material which is preferably selected so that it will have little, if any, damaging effect upon the quality of the metal, even though it may be dissolved therein to a slight extent; for example, in conjunction with the melting of aluminum a lining of aluminum oxide is preferred. The depending neck portion is similarly provided with a lining 31 of the same material, the refractory material preferably projecting slightly above the bottom of the crucible as indicated at 32 to prevent foreign matter which may accumulate in the bottom of the crucible from being discharged therefrom. The molten metal is discharged through the refractory lining 31 of the depending neck portion, the opening 33 through the bottom member 11 and the conduit 34 which leads to the cooling chamber where the casting process takes place, indicated generally at 35. The conduit 34 is also provided with a refractory lining 36, the lining being made in a plurality of small pieces, as shown, for convenience in installation. At its upper end the member 34 is provided with a flange 37 which is bolted to the bottom member 11 by bolts 38 which also secure the flange 39 of the neck portion 29 in place. Suitable gaskets may be used to prevent leakage between the flanges and the bottom portion.

The crucible may be heated by any convenient means such as by induction heating or the resistance heating coils indicated diagrammatically at 40 and 41 and disposed between the refractory lining 30 and the metallic shell 28. The lead-in wires 42 and 43 pass through the wall of the pressure chamber 10, the arrangement shown in Fig. 4 and to be described in greater detail below be-

ing employed to prevent the escape of gas under pressure around the lead-in wires and from the container. To control the temperature of the metal during its passage through the discharge conduits, separate heating coils 44 and 45, each provided with individual lead-in wires, are employed. Preferably the heating current for these coils is independently controllable so that the temperature of the crucible can be controlled by the coils 40 and 41, the temperature of the initial portion of the discharge conduit may be controlled by the coil 44 and the temperature of the end portion of the discharge conduit may be controlled by the coil 45. The heating effect of the several coils may be regulated by means of conventional rheostats or other similar devices not shown.

While the metal may be melted in the crucible, it is more convenient to melt the metal in another furnace and supply the molten metal to the crucible so that the crucible can be intermittently charged with molten metal without interrupting the discharge of metal under pressure therefrom. To this end, I have provided the charging mechanism associated with the upper portion of the pressure chamber. This preferably comprises a funnel shaped member 50 provided with a refractory lining 51 and adapted to receive molten metal from another furnace or ladle. The member 50 leads to a valve 52 which controls communication with the enlarged chamber 53, also having a refractory lining 54, and communicating through valve 55 with the conduit 56 which is adapted to discharge into the crucible 25. The conduit 56 has a lining 57 of refractory material extending through an opening 58 in the top closure member 12 and the conduit and valve member 55 are provided with flanges 59 and 60, respectively, which are bolted together and to the member 12 as by bolts 61, gaskets of other suitable packing means being provided to prevent the escape of gases under pressure between the respective flanges and the surfaces of the member 12.

In operation the valve 55, shown open in the drawing, is normally closed. When it is desired to charge the crucible 25, the valve 52 is opened and a charge of molten metal poured through the funnel 50 into the chamber 53. Then air or other suitable gas under pressure is admitted to the chamber 53 above the level of molten metal therein through the pipe 62 which is provided with a suitable pressure gauge 63 and control valve 64. The gas is admitted until the pressure in the chamber 53 equals or slightly exceeds the pressure in the large pressure chamber 10, which is indicated by gauge 65. Thereupon the valve 55 is opened and the molten metal in the chamber 53 is discharged into the crucible 25. Because of the relatively small size of the pressure chamber 53, it is unnecessary to balance the fluid pressures on the inside and outside of the chamber as the chamber walls may be made of sufficient strength to resist the internal pressures. Further, the molten metal remains in the chamber for only a short time and the metallic outer walls have an opportunity to cool in between charging operations. By this means, molten metal may be discharged continuously from the crucible 25, it being unnecessary to interrupt the operation in order to replenish the supply of metal within the crucible.

Depending upon the metal employed and the type of material being produced, the pressures

within the pressure chamber 10 and on the molten metal within the crucible 25 may be varied from moderate pressures of the order of one or two hundred pounds per square inch to rather high pressures on the order of twelve hundred or fifteen hundred pounds per square inch. By reason of the fact that the pressures are applied equally on the inside and outside of the crucible, no destructive forces are imposed on the crucible and thus the high pressures can be handled with safety.

The metal under pressure is discharged through the conduits heretofore described into the discharge zone indicated generally at 35 which constitutes a separate unit bolted to the flange 67 at the end of the conduit 36. It is in this unit that the metal is given its desired shape and where the solidification takes place. This may be termed the cooling, casting or extruding unit and comprises an inner passageway or die 78 which has the cross-sectional shape throughout the greater portion of its length of the ultimate product, in the present example a round wire being illustrated, and which is provided with a flared portion 79 for connection with the end of the conduit 36. The member 78 is surrounded by a reinforcing member 80 and the temperature of the members 78 and 80 is controlled by immersing them in a bath of molten material having a melting point suitable for the purpose. In conjunction with the production of aluminum wire, I prefer to employ a bath of molten lead indicated at 81, the lead being heated by a suitable electric heating coil 82. The molten lead provides a means for accurately controlling the temperature in the casting zone and avoiding abrupt changes in temperature. By this means the temperature can be controlled and correlated with the speed of discharge so that the liquid metal flowing through the member 78 will congeal and become plastic and then solid after it has been given the desired cross-sectional shape but before it is discharged from the end of the member 78. The passageway 78 may be of uniform cross-section throughout, or it may be tapered slightly in accordance with the shrinkage characteristic of the metal.

By so controlling the temperature, the cross-sectional shape can be formed without requiring excessive pressures and, inasmuch as the member 78 is of considerable length, as distinguished from a die of the type used in ordinary extrusion operations, slight variations in temperature will not prevent the metal from solidifying within the member 78 so that it can be withdrawn, for example, by the rolls 83 disposed closely adjacent the discharge end of the member 78. As shown in Fig. 3, the rolls 83 are provided with grooves conforming to the desired cross-sectional contour of the discharged wire and, if desired, the metal can be discharged from the die member 78 at an elevated temperature while it is still in a somewhat plastic condition, in which case the rolls may be used to effect a further reduction in cross-sectional area or final shaping of the material. If desired, the metal, while still hot, may be drawn through a die (not shown) disposed near the point of discharge to work, size or reduce the extruded material.

As noted above, under some conditions rather high pressures may be required in carrying out the continuous casting operation and, therefore, it is important that effective seals be produced where the wires 42 and 43 pass through the walled pressure chamber 10. To this end, I have pro-

vided the structure shown in Fig. 4 of the drawing and comprising a water jacketed tube 85 securely bolted to the wall of the chamber 10 as by bolts 86, a gasket 87 being employed to prevent leakage between the tube and the walled pressure chamber. The tube may be cooled by water or other suitable cooling medium passing through the water jacket space 88 and being supplied to the water jacket through the pipe 89, the liquid being discharged from the jacket through the pipe 90.

The wire 42 passes through the tube 85 and is insulated therefrom by being encased within a tube of a heat resisting insulating material 91. This material may be a suitable plastic insulation such as a Bakelite composition, or vitreous materials such as glass may be employed. The insulating material, whatever it is, is sealed to the wire so that the gas under pressure within the container cannot leak between the wire 42 and its sheath of insulating material 91.

To prevent leakage between the tube 85 and the sheath of insulated material 91, any suitable packing means may be employed, this being disposed adjacent the outer end of the tube away from the pressure chamber, a simple and effective construction comprising a packing gland member 92 having a flange 93 which is bolted to the flange 94 of the tube 85 by a number of bolts 95. The interior of the packing gland is filled with packing material 96 which may be compressed by the bolts 95.

By this arrangement a sturdy and effective seal can be made between the wires and the wall of the pressure chamber. The wire itself is sealed within a sheath of insulating material and the seal between the insulating material and the tube is made in a zone spaced away from the pressure chamber so that all of the parts, including the wire, the sheath of insulating material, the tube, the packing gland and the packing material may be maintained at reasonably low temperatures regardless of the temperature within the pressure chamber. Thus, as the temperature where the actual seal is made is fairly low and may be kept quite uniform, differences in coefficients of expansion of the sheath material involved will not cause any difficulties and an effective seal can be made.

To summarize the operation of the apparatus and the steps of the method, the crucible 25 may be charged with a molten metal through the charging mechanism disposed above the pressure chamber. The heating current supplied to the coils of the crucible is regulated to maintain the molten metal at the desired temperature above its melting point and gas under pressure is admitted through the tube 97 until the desired pressure indicated on the gauge 98 is reached. Under these circumstances, the molten metal is forced outwardly through the conduit 31 into the cooling or casting unit 35. The temperature of the metal as it flows through the conduit may be regulated by the various heating coils 44 and 45.

The metal, while in the liquid state, is caused to take its desired cross-sectional shape, the section being reduced by the tapered portion 79 of the conduit 78. Thereafter, the fluid pressure exerted upon the metal in the crucible causes it to flow along the conduit 78 without substantial change in cross-sectional shape, except for shrinkage and during the time that the metal is flowing through the bore of the member 78 the

metal is cooled sufficiently to cause it to become either plastic or solid, as desired. The cooling of the metal is controlled by immersing the conduit 78 in a cooling bath, the temperature of which may be regulated as by the electric heating coil 82.

After the material has become solidified or at least plastic to the extent that it can be handled, it is withdrawn from the conduit 78, a flame of reducing character 99 preferably being employed to prevent oxidation at this point. Thereafter, the material is passed between the rolls 83 which may function either to merely withdraw the metal from the conduit 78, or, in addition, to effect some additional working of the metal. In this last arrangement, the metal may be discharged from the conduit 78 while in the plastic rather than solid state, or at least at a temperature where it may be worked readily. From the rolls 83 the metal is discharged onto any suitable run-out table or wound on a reel or otherwise suitable handled. A conveyor roll 100 may be employed to support the metal before the reeling operation and, if desired, the metal after passing between the rolls 83 may be cooled by jets of water, steam or other medium indicated at 101.

In operation, the pressure within the pressure chamber is correlated with the cross-sectional area of the shape being produced and the friction through the member 78 so that the metal will be forced through the member 78 at the desired speed. The speed and temperature, further, must be correlated so that the metal will be cooled and solidified during its passage through the member 78 after the metal has been given the desired cross-sectional shape, so that the metal may be withdrawn by the rolls 83 without breaking the wire, rod, strip, or the like, being produced. Because of the comparatively great length of the bore of the member 78, the speeds and temperatures do not need to be controlled with an exceptionally high degree of accuracy for variations will merely cause differences in the points where the solidification of the metal takes place, which variations do no harm so long as the metal becomes solid within the uniform or slightly tapered bore of the member 78. The pressures, speeds and temperatures in the cooling may vary, depending upon the materials involved and the cross-sectional area and shape of the ultimate product.

In the foregoing specification, I have disclosed a preferred form of my invention both as to method and apparatus. Various modifications in both my method and apparatus may be made without departing from the spirit and scope of my invention. Accordingly, it is to be understood that my patent is not limited to the preferred form described in the foregoing specification or in any manner other than by the scope of the appended claims when given the range of equivalents to which my patent may be entitled.

I claim:

1. In an apparatus of the type described, a pressure chamber, means for cooling the pressure chamber, a crucible disposed within said pressure chamber, means for supplying a gas under greater than atmospheric pressure to said pressure chamber to force molten material out of said crucible, means for heating said crucible, means for charging said crucible from a supply at a lower pressure without releasing the pressure within said pressure chamber, and a conduit extending from the interior of said crucible to the exterior of said pressure chamber for continu-

ously discharging the contents of said crucible under pressure.

2. In an apparatus of the type described, a pressure chamber, means for cooling the pressure chamber, a crucible disposed within said pressure chamber, means for supplying a gas under greater than atmospheric pressure to said pressure chamber, means for charging said crucible without releasing the pressure within said pressure chamber, and a conduit extending from the interior of said pressure chamber for discharging the contents of said crucible under pressure, separately controllable heating means for said crucible and said conduit, said conduit terminating in a section having a cross-section corresponding to the cross-section of the material to be produced, means for cooling said section to solidify metal therein, and a pair of rolls disposed adjacent the end of said section for withdrawing solidified metal therefrom.

3. An apparatus for forming metal rod, wire, strip and the like comprising a crucible for containing molten metal, means for applying gas pressure to the surface of the metal in the crucible, a conduit leading from the crucible for discharging molten metal under pressure therefrom, separately controllable heating means for said crucible and said conduit, a die adapted to receive molten metal from said conduit, said die having a flared mouth portion connected to said conduit and an elongated open-ended portion having substantially the cross-sectional shape of the finished product, and means for cooling said elongated portion comprising a bath of molten metal surrounding said elongated portion.

4. In an apparatus of the type described, a pressure chamber, means for cooling the pressure chamber, a crucible disposed within said pressure chamber, means for supplying a gas under greater than atmospheric pressure to said pressure chamber, means for charging said crucible without releasing the pressure within said pressure chamber, and a conduit extending from the interior of said crucible to the exterior of said pressure chamber for discharging the contents of said crucible under pressure of said gas, separately controllable heating means for said crucible and said conduit, said conduit terminating in an open-ended section having a cross-section corresponding to the cross-section of the material to be produced, and means for cooling said section to solidify metal therein.

5. In an apparatus of the type described, a pressure chamber, a crucible disposed within said pressure chamber, means for supplying a gas under greater than atmospheric pressure to said pressure chamber, means for charging said crucible without releasing the pressure within said pressure chamber, and a conduit extending from the interior of said crucible to the exterior of said pressure chamber for discharging the contents of said crucible under pressure, separately controllable heating means for said crucible and said conduit, said conduit terminating in an open-ended section having a cross-section corresponding to the cross-section of the material to be produced, and means for cooling said section to solidify metal therein.

6. In an apparatus of the type described, a pressure chamber, means for cooling the pressure chamber, a crucible disposed within said pressure chamber, means for supplying a gas under greater than atmospheric pressure to said pressure chamber, means for heating said

crucible, means for charging said crucible without releasing the pressure within said pressure chamber, and a conduit extending from the interior of said crucible to the exterior of said pressure chamber for discharging the contents of said crucible under pressure, said conduit terminating in an open ended section having a cross-section corresponding to the cross-section of the material to be produced, and means for cooling said section to solidify metal therein.

7. An apparatus for forming metal rod, wire, strip and the like comprising a crucible for containing molten metal, means for applying gas pressure to the surface of the metal in the crucible, a conduit leading from the crucible for discharging molten metal under pressure therefrom, separately controllable heating means for said crucible and said conduit, and a die adapted to receive molten metal from said conduit, said die having a flared mouth portion connected to 20

said conduit and an elongated, open-ended portion having substantially the cross-sectional shape of the finished product, and means for cooling said elongated portion.

5 8. The method of making metallic rod, wire, strip and the like, which includes the steps of continuously discharging molten metal from a crucible by gas pressure, intermittently charging the crucible with metal from a supply at substantially atmospheric pressure without substantially affecting the discharge of metal under pressure therefrom, continuously conducting the discharged metal under pressure into a cooling zone, causing the metal, while in the molten state, to take the desired cross-sectional shape in 10 said cooling zone, cooling the metal in said cooling zone and causing the metal to substantially solidify in said cooling zone, and continuously discharging the metal therefrom.

JOSEPH B. BRENNAN.